

## UNITED STATES PATENT OFFICE

2,416,773

## STABILIZED DIAZOTYPE PHOTOPRINTING MATERIALS

Maximilian K. Reichel, Easton, Pa., assignor to  
General Aniline & Film Corporation, New York,  
N. Y., a corporation of Delaware

No Drawing. Application January 4, 1945,  
Serial No. 571,352.

6 Claims. (Cl. 95—6)

1

This invention relates to the stabilization of photo-printing materials having light sensitive layers which are produced by the incorporation of a diazo compound as the light-sensitive medium onto the surface of a suitable carrier base. More particularly, it refers to the stabilization of so-called dry-development diazotype light-sensitive layers wherein the diazo compound is incorporated into the light sensitive layer together with an azo dyestuff coupling component. As diazo compounds for such dry-development or two-component diazotype light-sensitive layers, the most suitable have been found to be those which are derived from ortho- or para-amino-naphthols or aromatic paradiamines, particularly N-mono- or di-substituted aromatic paradiamines.

Various processes are known for the preparation of light-sensitive layers which depend upon the use of a diazo compound as the light-sensitive medium, and various materials have been employed for the carrier of the light-sensitive layer, including textiles, paper, cellulosic films, and glass and metal surfaces. The sensitized carrier is exposed to light under a transparent original which it is desired to reproduce and the diazo compound is decomposed in the areas unprotected by the outline of the original. The undecomposed diazo compound in the protected areas is then used to develop the image of the original by coupling the said diazo compound in an alkaline atmosphere with an azo dyestuff coupling component.

In the two-component layers which contemplate the incorporation of the coupling component into the light-sensitive layer with the diazo compound, the development of the dyestuff forming the image is effected by bringing the exposed light-sensitive layer into contact with gaseous ammonia. This is known as the dry developing process. The dyestuff components, as applied on the carrier are relatively unstable and cannot be stored for long periods prior to use. The light-sensitive layers which carry the coupling component as well as the diazo compound in the light-sensitive layer are subject to premature coupling of the said dyestuff components as well as decomposition of the diazo compound upon long storage.

Many attempts have been made to obtain more stable coating solutions and to render the light-sensitive layers produced therefrom less sensitive to deterioration without impairing the light-sensitive qualities of the diazo compound upon which the production of accurate images from the

2

original depends. These attempts have hitherto been relatively unsuccessful. It is therefore the object of this invention to provide coating solutions and light-sensitive layers, using diazo compounds as the light-sensitive medium which can be stored for long periods prior to use and will be stable during storage, even under unfavorable conditions.

I have found that coating solutions and the light-sensitive layers prepared therefrom can be stabilized against decomposition of the light-sensitive material and premature coupling of the dyestuff components by adding to the coating solution, a compound of the class of sulfonated ortho-hydroxy-carboxylic acids of the benzene or naphthalene series.

Examples of such compounds are:

5-sulfo-salicylic acid  
5-sulfo-o-cresotic acid  
6-sulfo-2-hydroxy-3-naphthalene-carboxylic acid  
8-sulfo-2-hydroxy-3-naphthalene-carboxylic acid

Diazotype light-sensitive layers which have been stabilized by addition of compounds of the above class show greatly improved keeping qualities and are stable against decomposition or deterioration for much longer periods of storage than hitherto possible when using the same diazo light-sensitive compositions without these stabilizers. The following examples illustrate the invention but they are not intended to limit it thereto. The parts are by weight unless otherwise stated.

## Example 1

35 A coating solution (A) was made up as follows:

|                                                                         | Parts |
|-------------------------------------------------------------------------|-------|
| Sulfate of the diazo compound obtained from<br>40 p-amino-diphenylamine | 14.6  |
| Citric acid                                                             | 100   |
| Acetoacetanilide                                                        | 9     |
| Thiourea                                                                | 45    |

were dissolved in 100 cc. of water. Another coating solution (B) was made up containing the same ingredients as in (A) except that 50 parts citric acid and 44 parts 5-sulfo-salicylic acid were substituted for the 100 parts of citric acid. These solutions were then separately spread on strips of paper, fabric, and film by the usual coating method for the production of diazo-type light-sensitive layers, using a doctor blade to insure a thin even coating. After storage at room temperature for several months, the stability of the sensitized materials of A and B was tested by ex-

posing a test piece to light under a suitable diazoitive and developing the image by application of ammonia gas. The resulting image reproduced on the light-sensitive layer containing the 5-sulfo-salicylic acid (solution B) was compared with the image reproduced under the same conditions on a light-sensitive layer made from the coating composition (A) and containing no 5-sulfo-salicylic acid which latter had been stored under the same conditions for the same length of time. The background, and consequently the contrast of the image, reproduced on the light-sensitive layer made in accordance with this example, is superior to that of the sample which does not contain the 5-sulfo-salicylic acid in the light-sensitive layer.

*Example 2*

The composition of the coating solutions A and B was the same as in Example 1, but as a stabilizer 47 parts 5-sulfo-o-cresotic acid per liter were used instead of the 5-sulfo-salicylic acid. The coatings of A and B and the storage and testing procedures were the same as in Example 1. The stability of the coating made according to this example was found to be superior to that of the coating made from a solution not containing 5-sulfo-o-cresotic acid as a stabilizer.

*Example 3*

The composition of the coating solutions A and B was the same as in Example 1, but as a stabilizer 53.5 parts of 8-sulfo-2-hydroxy-3-naphthalene-carboxylic acid per liter were used instead of the 5-sulfo-salicylic acid. The coating, storage, and testing procedures were the same as in Example 1. The stability of the coating made according to this example was found to be superior to that of the coating made from solution A not containing 8-sulfo-2-hydroxy-3-naphthalene-carboxylic acid as a stabilizer.

*Example 4*

A coating solution was made up as follows:

|                                                                                               | Parts |
|-----------------------------------------------------------------------------------------------|-------|
| Zinc chloride double salt of the diazo compound obtained from N,N-dimethyl-p-phenylenediamine | 12.5  |
| Citric acid                                                                                   | 100   |
| 2,3-dihydroxy-naphthalene                                                                     | 5.9   |
| Thiourea                                                                                      | 45.0  |
| Sodium salt of the naphthalene-1,3,6-trisulfonic acid                                         | 32.5  |
| Aluminum sulfate                                                                              | 6.9   |

were dissolved in 1000 cc. of water (solution A). Another coating solution (B) was made up containing the same ingredients as in solution (A) except that 50 parts citric acid and 44 parts of 5-sulfo-salicylic acid were substituted for the 100 parts of citric acid. Solutions A and B were then separately spread on strips of paper, fabric, and film by the usual coating method in the same manner as described in Example 1. The light-sensitive layer thus produced was then stored at room temperature for several months and its stability then tested by observing the appearance of color in the light-sensitive layer due to premature coupling of the dye components and by comparison of its light-sensitive qualities with those of a test sample prepared and treated in the same manner as the light-sensitive layer of this example but omitting the 5-sulfo-salicylic acid as a stabilizer. When so tested, it was found that the light-sensitive layer made in accordance with

this example shows no discoloration due to premature coupling of the dye components after the storage period, whereas, the light-sensitive layer not having the 5-sulfo-salicylic acid as a stabilizing agent, under the same conditions, shows a considerable amount of coloring, due to premature coupling.

*Example 5*

The composition of the coating solution A and B was the same as in Example 4, but as a stabilizer, 47 parts of 5-sulfo-o-cresotic acid per liter were used instead of the 5-sulfo-salicylic acid. The coating, storage, and testing procedures were the same as in Example 4. The stability of the coating made according to this example (B) was found to be superior to that of a coating made from solution (A) not containing 5-sulfo-o-cresotic acid as a stabilizer.

*Example 6*

A coating solution was made up as follows:

|                                                                                               | Parts |
|-----------------------------------------------------------------------------------------------|-------|
| Zinc chloride double salt of the diazo compound obtained from N,N-diethyl-p-phenylene-diamine | 14    |
| Citric acid                                                                                   | 100   |
| 1-phenyl-3-methyl-pyrazolone                                                                  | 8     |
| Thiourea                                                                                      | 45    |

were dissolved in 1000 cc. of water (solution A). Another coating solution (B) was made up containing the same ingredients as in solution A except that 50 parts of citric acid and 47 parts of 5-sulfo-o-cresotic acid were substituted for the 100 parts of citric acid. Solutions A and B are then separately spread on strips of paper, fabric, and film by the usual coating method in the same manner as described in Example 1. The light-sensitive layer thus produced was then stored at room temperature for several months and its stability then tested in the same manner as in Example 1. The stability of the coating made according to this example was found to be superior to that of the coating made from a solution (A), not containing 5-sulfo-o-cresotic acid.

*Example 7*

A coating solution was made up as follows:

|                                                 | Parts |
|-------------------------------------------------|-------|
| 2,1 - diazo-hydroxy-naphthalene-5-sulfonic acid | 14.0  |
| Citric acid                                     | 100   |
| Nickel sulfate                                  | 31.5  |
| Phloroglucine                                   | 4.9   |
| Thiourea                                        | 20.0  |

lene carboxylic acid per liter were used instead of the 5-sulfo-o-cresotic acid. The coating, storage and testing procedures are the same as in Example 1. The stability of the coating made according to this example was found to be superior to that of the coating made from solution A not containing 6-sulfo-2-hydroxy-3-naphthalene-carboxylic acid as a stabilizer.

Having now fully described my invention and having set forth the best manner in which to practice it, what I claim as new is:

1. Photoprinting materials comprising light-sensitive layers on a suitable base containing in the light-sensitive layer a diazo compound suitable for forming a stable two-component diazo-type layer, an azo dye coupling component and a member of the class consisting of sulfonated ortho-hydroxy-carboxylic acids of the benzene and naphthalene series.

2. Photoprinting materials comprising light-sensitive layers on a suitable base containing in the light-sensitive layer a diazo compound derived from an aromatic paradiamine, an azo dye coupling component and a member of the class consisting of sulfonated ortho-hydroxy-carboxylic acids of the benzene and naphthalene series.

3. Photoprinting materials comprising light-sensitive layers on a suitable base containing in the light-sensitive layer a diazo compound derived from an ortho-aminonaphthol compound, an azo dye coupling component and a member of

the class consisting of sulfonated ortho-hydroxy-carboxylic acids of the benzene and naphthalene series.

4. Photoprinting materials comprising light-sensitive layers on a suitable base containing in the light-sensitive layer a diazo compound derived from an aromatic paradiamine, an azo dye coupling component and 5-sulfo-salicylic acid.

5. Photoprinting materials comprising light-sensitive layers on a suitable base containing in the light sensitive layer a diazo compound derived from an aromatic paradiamine, an azo dye coupling component and 8-sulfo-2-hydroxy-3-naphthalene-carboxylic acid.

6. Photoprinting materials comprising light-sensitive layers on a suitable base containing in the light-sensitive layer, a diazo compound derived from an ortho-aminonaphthol compound, an azo dye coupling component and 5-sulfo-o-cresotic acid.

MAXIMILIAN K. REICHEL.

#### REFERENCES CITED

The following references are of record in the 25 file of this patent:

#### UNITED STATES PATENTS

| Number    | Name                 | Date          |
|-----------|----------------------|---------------|
| 1,760,780 | Schmidt et al. ----- | May 27, 1930  |
| 1,811,029 | Schmidt et al. ----- | June 23, 1931 |
| 1,845,989 | Schmidt et al. ----- | Feb. 16, 1932 |